# EUROPEAN PATENT APPLICATION

(11) **EP 4 775 654 A1**
(43) Date of publication of application: **15.07.2026**
(21) Application number: 24874700.8
(22) Date of filing: 03.10.2024
(51) Int. Cl.: C10M 105/06, C10N 20/00, C10N 20/02, C10N 30/06, C10N 40/30

(54) **REFRIGERANT OIL, WORKING FLUID COMPOSITION, AND METHOD FOR REDUCING FRICTION COEFFICIENT OF SLIDING PART**

(30) Priority: 04.10.2023 JP 2023172833
(71) Applicant: ENEOS CORPORATION, Chiyoda-ku Tokyo 100-8162 (JP)
(72) Inventor: NARA Fumiyuki, Tokyo 100-8162 (JP); ANDO Makoto, Tokyo 100-8162 (JP); OGATA Hidetoshi, Tokyo 100-8162 (JP); MIZUTANI Yuya, Tokyo 100-8162 (JP); TAKAKI Tomohiro, Tokyo 100-8162 (JP)
(74) Representative: Grünecker Patent- und Rechtsanwälte PartG mbB
(86) International application number: PCT/JP2024/035478
(87) International publication number: WO 2025/075100

(57) **Abstract**

A refrigerating machine oil comprising an alkylbenzene and a hydrocarbon oil other than the alkylbenzene, the hydrocarbon oil having a refractive index at 20°C of 1.445 or less.

## Description

### Technical Field

The present disclosure relates to a refrigerating machine oil, a working fluid composition, and a method for reducing a coefficient of friction of a sliding portion.

### Background Art

Refrigerators, freezers, air conditioners (such as car air conditioners and room air conditioners), water heaters, and other refrigeration machines are provided with a compressor for circulating a refrigerant in a refrigeration cycle. The compressor is filled with a refrigerating machine oil for lubricating sliding members.

Various types of base oils are known as a base oil that is a main component of the refrigerating machine oil, and an appropriate base oil is selected depending on desired properties. For example, Patent Literature 1 discloses a lubricant composition for use in a refrigeration machine operated with a refrigerant composed of at least one component of an HC (hydrocarbon) group, the lubricant composition comprising an alkylbenzene oil containing at least 90% by weight of a linear alkylbenzene selected from linear alkyl groups having paraffin side chains having 10 to 13 carbon atoms, having an average molecular weight of 239 to 244 g/mol, and having a viscosity between 4.0 cSt and 5.0 cSt at a temperature of 40°C.

### Citation List

### Patent Literature

[Patent Literature 1] Japanese Patent No. 5683068

### Summary of Invention

### Technical Problem

According to studies by the present inventors, a refrigerating machine oil containing an alkylbenzene as disclosed in Patent Literature 1 does not necessarily have sufficient low-friction properties, and there is room for improvement.

Therefore, one aspect of the present invention is to effectively reduce a coefficient of friction of a sliding portion by using a refrigerating machine oil containing an alkylbenzene.

### Solution to Problem

As a result of studies by the present inventors on a method for reducing a coefficient of friction of a sliding portion by mixing, with an alkylbenzene, a hydrocarbon oil other than the alkylbenzene, it has been found that by mixing a hydrocarbon oil having a specific refractive index, the coefficient of friction of the sliding portion can be effectively (additively or synergistically) reduced as compared with the case where the alkylbenzene is used alone. The present invention includes the following aspects.
[1] A refrigerating machine oil comprising an alkylbenzene and a hydrocarbon oil other than the alkylbenzene, the hydrocarbon oil having a refractive index at 20°C of 1.445 or less.
[2] The refrigerating machine oil according to [1], wherein a refractive index (n20) of the hydrocarbon oil at 20°C and a kinematic viscosity (KV100) at 100°C satisfy the following formula: $1.420 \leq n 20 - 0.002 \times KV 100 \leq 1.445 .$
[3] The refrigerating machine oil according to [1] or [2], wherein a kinematic viscosity of the refrigerating machine oil at 40°C is 5 mm²/s or less.
[4] A working fluid composition comprising the refrigerating machine oil according to any one of [1] to [3], and a refrigerant.
[5] A method for reducing a coefficient of friction of a sliding portion by using a refrigerating machine oil containing an alkylbenzene, the method comprising mixing, with the alkylbenzene, a hydrocarbon oil other than the alkylbenzene, the hydrocarbon oil having a refractive index at 20°C of 1.445 or less, thereby reducing the coefficient of friction of the sliding portion.

### Advantageous Effects of Invention

According to one aspect of the present invention, a coefficient of friction of a sliding portion can be effectively reduced by using a refrigerating machine oil containing an alkylbenzene.

### Description of Embodiments

Hereinafter, embodiments of the present invention will be described in detail. One embodiment of the present invention is a refrigerating machine oil comprising an alkylbenzene and a hydrocarbon oil other than the alkylbenzene, the hydrocarbon oil having a refractive index at 20°C of 1.445 or less (hereinafter also simply referred to as "hydrocarbon oil").

The alkylbenzene may be a linear alkylbenzene, and may also be a branched alkylbenzene. The linear alkylbenzene is an alkylbenzene in which a linear alkylating agent is bonded to a benzene ring. The linear alkyl group may be bonded to the benzene ring at any position of the alkyl group. The branched alkylbenzene is an alkylbenzene in which a branched alkylating agent is bonded to a benzene ring. The branched alkyl group may be bonded to the benzene ring at any position of the alkyl group.

The alkylbenzene is preferably a linear alkylbenzene from the viewpoint that the refrigerating machine oil tends to have low viscosity and that an effect of reducing a coefficient of friction by blending a hydrocarbon oil other than the alkylbenzene is easily obtained. The linear alkylbenzene may be a compound represented by the following formula (1). [Formula 1] In the formula, m and n are each independently an integer of 0 to 12, and are integers satisfying m + n = 7 to 12.

m and n may be integers that are each independently preferably an integer of 1 to 11, 1 to 10, 1 to 9, 1 to 8, 1 to 7, or 1 to 6, and that satisfy m + n = 8 to 12 or 9 to 12.

The alkylbenzene may be a mixture of two or more linear alkylbenzenes represented by formula (1). The alkylbenzene may contain two or more linear alkylbenzenes in which m and n in formula (1) are each independently integers of 1 to 6 and satisfy m + n = 9 to 12, and may preferably contain the two or more linear alkylbenzenes as main components. A total content of the two or more linear alkylbenzenes is preferably 40% by mass or more, 50% by mass or more, 60% by mass or more, 80% by mass or more, 90% by mass or more, or 95% by mass or more, based on the total amount of the alkylbenzene.

An average molecular weight of the alkylbenzene (preferably the linear alkylbenzene) may be 180 or more, 200 or more, or 230 or more, and may be 280 or less, 260 or less, or 250 or less.

A kinematic viscosity of the alkylbenzene (preferably the linear alkylbenzene) at 40°C may be 10 mm²/s or less, 5 mm²/s or less, 4.8 mm²/s or less, 4.6 mm²/s or less, or 4.5 mm²/s or less, and may be 1 mm²/s or more, 2 mm²/s or more, 3 mm²/s or more, or 4 mm²/s or more. A kinematic viscosity of the alkylbenzene (preferably the linear alkylbenzene) at 100°C may be 0.5 mm²/s or more, 1 mm²/s or more, 1.2 mm²/s or more, or 1.3 mm²/s or more, and may be 4 mm²/s or less, 3 mm²/s or less, 2 mm²/s or less, 1.8 mm²/s or less, 1.7 mm²/s or less, or 1.6 mm²/s or less. The kinematic viscosity in the present specification means a kinematic viscosity measured in conformity with JIS K2283:2000.

A refractive index of the alkylbenzene (preferably the linear alkylbenzene) at 20°C may be 1.470 or more or 1.480 or more, and may be 1.500 or less, 1.495 or less, or 1.490 or less. The refractive index in the present specification means a refractive index measured in conformity with JIS K0062:1992.

A content of the alkylbenzene (preferably the linear alkylbenzene) may be 10% by mass or more, 20% by mass or more, 30% by mass or more, or 40% by mass or more, and may be 90% by mass or less, less than 90% by mass, 85% by mass or less, 80% by mass or less, 70% by mass or less, or 60% by mass or less, based on the total amount of the refrigerating machine oil.

A method for producing the alkylbenzene is arbitrary and is not particularly limited. The alkylbenzene can be produced, for example, by bringing an aromatic compound into contact with an alkylating agent in the presence of a catalyst. Specific examples of the aromatic compound as a raw material include benzene, toluene, xylene, ethylbenzene, methylethylbenzene, diethylbenzene, and mixtures thereof.

Examples of the linear alkylating agent for obtaining a linear alkylbenzene include a linear paraffin separated from petroleum fractions such as kerosene and light oil, a linear olefin obtained by olefinating a linear paraffin with a catalyst, and a linear olefin obtained by polymerizing ethylene, which are linear paraffin or olefin compounds having 8 to 40 carbon atoms. Examples of the branched alkylating agent for obtaining a branched alkylbenzene include branched olefins having 6 to 40 carbon atoms obtained by polymerization of lower monoolefins such as ethylene, propylene, butene, and isobutylene; branched olefins having 6 to 40 carbon atoms obtained by thermal decomposition of waxes, heavy oils, petroleum fractions, polyethylene, polypropylene, and mixtures thereof; and the like, and preferably include propylene oligomers.

Examples of the alkylation catalyst used for alkylation include known catalysts such as Friedel-Crafts catalysts such as aluminum chloride and zinc chloride; and acidic catalysts such as sulfuric acid, phosphoric acid, silicotungstic acid, hydrofluoric acid, and activated clay.

When a linear alkylbenzene represented by formula (1) is used, the linear alkylbenzene represented by formula (1) may be separated from the alkylated aromatic compound obtained as described above and used, and it is preferable to directly alkylate benzene using, as the alkylating agent, a linear paraffin, a linear chlorinated paraffin, a linear olefin such as an α-olefin, or the like. The linear alkylbenzene represented by formula (1) in which m + n = 9 to 12 produced using a linear alkylating agent having 10 to 13 carbon atoms is commercially available and is preferable from the viewpoint of economy.

The hydrocarbon oil other than the alkylbenzene has a refractive index at 20°C of 1.445 or less. In one embodiment, since the hydrocarbon oil has a lower refractive index than the above alkylbenzene, the hydrocarbon oil and the alkylbenzene can also be distinguished from each other on the basis of the refractive index. From the viewpoint of further reducing a coefficient of friction, the refractive index of the hydrocarbon oil at 20°C may preferably be 1.444 or less or 1.443 or less, and more preferably 1.442 or less, 1.441 or less, 1.440 or less, or 1.439 or less. The refractive index of the hydrocarbon oil at 20°C may be 1.420 or more, 1.425 or more, 1.430 or more, 1.432 or more, or 1.435 or more.

The hydrocarbon oil may be appropriately selected from hydrocarbon oils having the above refractive indices. Examples of the hydrocarbon oil include mineral oil hydrocarbon oils and synthetic hydrocarbon oils. The hydrocarbon oil may be used alone or in combination of two or more thereof.

Examples of the mineral oil hydrocarbon oil include normal paraffinic, isoparaffinic, or naphthenic hydrocarbon oils (refined mineral oils) obtained by refining a crude oil or a distillation residue oil as a raw material by appropriately combining ordinary petroleum refining treatments (such as solvent deasphalting, solvent extraction, hydrocracking, solvent dewaxing, catalytic dewaxing, hydrotreating, sulfuric acid washing, clay treatment, and distillation, and the like).

Examples of the synthetic hydrocarbon oil include, for example, poly-α-olefins or hydrogenated products thereof, α-olefins and other olefins, and isoparaffins. The synthetic hydrocarbon oil is preferably an α-olefin or an isoparaffin.

The number of carbon atoms of the olefin may be 12 or more, 13 or more, or 14 or more, and may be 30 or less, 25 or less, or 20 or less. The olefin is preferably a linear olefin such as an α-olefin. The isoparaffin may be an isoparaffin obtained by refining a component containing normal paraffins obtained by a dewaxing step in a petroleum refining process or by Fischer-Tropsch synthesis, or a polymer of olefins such as ethylene, propylene, butylene, and diisobutylene, by appropriately combining hydrocracking, hydroisomerization, hydrodewaxing, hydrotreating, distillation, and the like.

From the viewpoint that a coefficient of friction can be further reduced, the hydrocarbon oil may preferably contain at least one hydrocarbon oil selected from the group consisting of normal paraffinic hydrocarbon oils, olefinic hydrocarbon oils, and isoparaffinic hydrocarbon oils, and may more preferably contain at least one hydrocarbon oil selected from the group consisting of linear olefinic hydrocarbon oils such as α-olefins and isoparaffinic hydrocarbon oils.

A kinematic viscosity of the hydrocarbon oil at 40°C may be 1 mm²/s or more, 1.5 mm²/s or more, or 2 mm²/s or more, and may be 5 mm²/s or less, 4 mm²/s or less, or 3 mm²/s or less. A kinematic viscosity of the hydrocarbon oil at 100°C may be 0.5 mm²/s or more, 0.7 mm²/s or more, or 0.9 mm²/s or more, and may be 2 mm²/s or less, 1.5 mm²/s or less, or 1.2 mm²/s or less.

A refractive index (n20) of the hydrocarbon oil at 20°C and a kinematic viscosity (KV100) at 100°C preferably satisfy the following formula: $1.420 \leq n 20 - 0.002 \times KV 100 \leq 1.445 .$ Hereinafter, a value of the expression "n20 - 0.002 × KV100" in the middle of the above formula is also referred to as an N value.

A lower limit of the N value in the above formula may be 1.421, 1.422, 1.423, 1.424, 1.425, 1.426, or 1.427. An upper limit of the N value in the above formula may be 1.444, 1.443, 1.442, 1.441, 1.440, 1.439, 1.438, or 1.437.

A %C_{A} (percentage of aromatic carbon) of the hydrocarbon oil may be 5 or less, 3 or less, 2 or less, 1 or less, or 0.5 or less. A %C_{N} (percentage of naphthenic carbon) of the hydrocarbon oil may be 50 or less, 30 or less, 20 or less, less than 20, 15 or less, 10 or less, or 5 or less. A %C_{P} (percentage of paraffinic carbon) of the hydrocarbon oil may be 50 or more, 70 or more, 80 or more, 90 or more, or 95 or more, and may be 100 or less, 95 or less, or 80 or less. The total of %C_{A}, %C_{N}, and %C_{P} is 100.

An R_{A} (average number of aromatic rings per molecule) of the hydrocarbon oil may be 0.5 or less, 0.2 or less, 0.1 or less, or 0.05 or less, and may be 0.00, and may be 0.00 or more. An R_{N} (average number of naphthenic rings per molecule) of the hydrocarbon oil may be 0.8 or less, 0.5 or less, 0.2 or less, or 0.1 or less, and may be 0.00, and may be 0.00 or more. An R₁ (average total number of rings per molecule = R_{N} + R_{A}) of the hydrocarbon oil may be 0.8 or less, 0.5 or less, 0.2 or less, or 0.1 or less, and may be 0.00, and may be 0.00 or more.

The %C_{A}, %C_{N}, %C_{P}, R_{A}, R_{N}, and R_{T} in the present specification mean values calculated by a method in conformity with ASTM D3238-17a (2017) "Standard Test Method for Calculation of Carbon Distribution and Structural Group Analysis of Petroleum Oils by the n-d-M Method". However, when an average molecular weight of the hydrocarbon oil is 250 or more, an average molecular weight calculated in conformity with ASTM D2502 or 2503 may be used as the average molecular weight, but when the average molecular weight of the hydrocarbon oil is less than 250, the value may not necessarily be reliable. Therefore, particularly when the average molecular weight of the hydrocarbon oil is less than 250, in accordance with the description in the section "3. Summary of Test Method" of the same test method, a molecular weight is experimentally determined, and the calculated average molecular weight is used. In this case, an average molecular weight calculated from a carbon number distribution (area %) obtained by gas chromatography (standard sample: n-paraffin) is used as the average molecular weight. From the viewpoint that further low-friction properties can be imparted, the average molecular weight of the hydrocarbon oil is preferably 430 or less, 350 or less, 300 or less, 250 or less, less than 250, or 220 or less, and from the viewpoint of reducing volatility and maintaining a flash point, preferably 140 or more, 150 or more, 160 or more, or 180 or more. In addition, if any of the calculated values of %C_{P}, %C_{A}, and %C_{N} is a negative value, the value is regarded as 0, and the remaining calculated values are corrected so that the total is 100 while maintaining the ratio. Among the above-described hydrocarbon oils, an olefin or a hydrocarbon oil containing an olefin is outside the application scope of the same test method and may not necessarily be reliable, and therefore, when the influence of the olefin cannot be ignored, the values are considered as reference values.

A content of the hydrocarbon oil may be 10% by mass or more, more than 10% by mass, 15% by mass or more, 20% by mass or more, 30% by mass or more, or 40% by mass or more, and may be 90% by mass or less, 80% by mass or less, 70% by mass or less, or 60% by mass or less, based on the total amount of the refrigerating machine oil.

A total content of the alkylbenzene and the hydrocarbon oil may be 50% by mass or more, 60% by mass or more, 70% by mass or more, 80% by mass or more, or 90% by mass or more, and may be 99% by mass or less, based on the total amount of the refrigerating machine oil.

In the refrigerating machine oil described above, by mixing, with the alkylbenzene, the hydrocarbon oil other than the alkylbenzene as described above, the coefficient of friction can be reduced as compared with the case where the alkylbenzene is used alone. That is, one embodiment of the present invention can also be said to be a method for reducing a coefficient of friction of a sliding portion by using a refrigerating machine oil containing an alkylbenzene, the method comprising mixing, with the alkylbenzene, a hydrocarbon oil other than the alkylbenzene, the hydrocarbon oil having a refractive index at 20°C of 1.445 or less, thereby reducing the coefficient of friction of the sliding portion. The sliding portion is a sliding portion in a refrigeration machine, and may be a sliding portion in a compressor of the refrigeration machine.

Another embodiment of the present invention can also be said to be a method for producing a refrigerating machine oil for reducing a coefficient of friction of a sliding portion by using a refrigerating machine oil containing an alkylbenzene, the method comprising mixing, with the alkylbenzene, a hydrocarbon oil other than the alkylbenzene, the hydrocarbon oil having a refractive index at 20°C of 1.445 or less.

The refrigerating machine oil may further contain, as an additive, an anti-wear agent (also referred to as an extreme-pressure agent) from the viewpoint of improving wear resistance. Examples of the anti-wear agent include phosphorus-containing anti-wear agents. Examples of the phosphorus-containing anti-wear agent include phosphoric esters, thiophosphoric esters, acidic phosphoric esters, amine salts of acidic phosphoric esters, chlorinated phosphoric esters, phosphite esters, amine salts of phosphite esters, phosphonic esters, and amine salts of phosphonic esters. The phosphorus-containing anti-wear agent is preferably one or two or more selected from phosphoric esters and thiophosphoric esters.

Examples of the phosphoric ester include trialkyl phosphates, trialkenyl phosphates, and triaryl phosphates. Examples of the trialkyl phosphate include tributyl phosphate, tripentyl phosphate, trihexyl phosphate, triheptyl phosphate, trioctyl phosphate, trinonyl phosphate, tridecyl phosphate, triundecyl phosphate, tridodecyl phosphate, tritridecyl phosphate, tritetradecyl phosphate, tripentadecyl phosphate, trihexadecyl phosphate, triheptadecyl phosphate, and trioctadecyl phosphate. An example of the trialkenyl phosphate is trioleyl phosphate. Examples of the triaryl phosphate include triphenyl phosphate, tricresyl phosphate, tri(ethylphenyl) phosphate, tri(butylphenyl) phosphate, trixylenyl phosphate, cresyl diphenyl phosphate, and xylenyl diphenyl phosphate. The phosphoric ester is preferably a triaryl phosphate, more preferably one selected from triphenyl phosphate and tricresyl phosphate, and still more preferably tricresyl phosphate.

Examples of the thiophosphoric ester include trialkyl phosphorothionates, trialkenyl phosphorothionates, and triaryl phosphorothionates. Examples of the trialkyl phosphorothionate include tributyl phosphorothionate, tripentyl phosphorothionate, trihexyl phosphorothionate, triheptyl phosphorothionate, trioctyl phosphorothionate, trinonyl phosphorothionate, tridecyl phosphorothionate, triundecyl phosphorothionate, tridodecyl phosphorothionate, tritridecyl phosphorothionate, tritetradecyl phosphorothionate, tripentadecyl phosphorothionate, trihexadecyl phosphorothionate, triheptadecyl phosphorothionate, and trioctadecyl phosphorothionate. An example of the trialkenyl phosphorothionate is trioleyl phosphorothionate. Examples of the triaryl phosphorothionate include triphenyl phosphorothionate, tricresyl phosphorothionate, trixylenyl phosphorothionate, cresyl diphenyl phosphorothionate, and xylenyl diphenyl phosphorothionate. The thiophosphoric ester is preferably triphenyl phosphorothionate.

Examples of the acidic phosphoric ester include monobutyl acid phosphate, monopentyl acid phosphate, monohexyl acid phosphate, monoheptyl acid phosphate, monooctyl acid phosphate, monononyl acid phosphate, monodecyl acid phosphate, monoundecyl acid phosphate, monododecyl acid phosphate, monotridecyl acid phosphate, monotetradecyl acid phosphate, monopentadecyl acid phosphate, monohexadecyl acid phosphate, monoheptadecyl acid phosphate, monooctadecyl acid phosphate, monooleyl acid phosphate, dibutyl acid phosphate, dipentyl acid phosphate, dihexyl acid phosphate, diheptyl acid phosphate, dioctyl acid phosphate, dinonyl acid phosphate, didecyl acid phosphate, diundecyl acid phosphate, didodecyl acid phosphate, ditridecyl acid phosphate, ditetradecyl acid phosphate, dipentadecyl acid phosphate, dihexadecyl acid phosphate, diheptadecyl acid phosphate, dioctadecyl acid phosphate, and dioleyl acid phosphate.

Examples of the phosphite ester include dibutyl phosphite, dipentyl phosphite, dihexyl phosphite, diheptyl phosphite, dioctyl phosphite, dinonyl phosphite, didecyl phosphite, diundecyl phosphite, didodecyl phosphite, dioleyl phosphite, diphenyl phosphite, dicresyl phosphite, tributyl phosphite, tripentyl phosphite, trihexyl phosphite, triheptyl phosphite, trioctyl phosphite, trinonyl phosphite, tridecyl phosphite, triundecyl phosphite, tridodecyl phosphite, trioleyl phosphite, triphenyl phosphite, and tricresyl phosphite.

Examples of the phosphonic ester include dialkyl phosphonoacetates, dialkyl hydroxymethyl phosphonates, dialkyl hydroxyethyl phosphonates, and dialkyl hydroxyundecyl phosphonates. An alkyl group in these phosphonic esters may be a linear or branched alkyl group having 1 to 20 carbon atoms.

Examples of the amine constituting the above amine salts include alkyl or alkenyl amines having 4 to 20 carbon atoms.

A content of the anti-wear agent (preferably the phosphorus-containing anti-wear agent) may be 0.1 % by mass or more, 0.5% by mass or more, or 1% by mass or more, and may be 5% by mass or less, 4% by mass or less, or 3% by mass or less, based on the total amount of the refrigerating machine oil.

The refrigerating machine oil may further contain other additives. Examples of the other additives include antioxidants, acid scavengers, metal deactivators, pour point depressants, detergents-dispersants, and antifoaming agents. A total content of the other additives may be 10% by mass or less or 5% by mass or less, based on the total amount of the refrigerating machine oil.

A kinematic viscosity of the refrigerating machine oil at 40°C may be 1 mm²/s or more, 1.5 mm²/s or more, or 2 mm²/s or more, and may be 20 mm²/s or less, 15 mm²/s or less, 10 mm²/s or less, 7 mm²/s or less, 5 mm²/s or less, or 4 mm²/s or less.

A kinematic viscosity of the refrigerating machine oil at 100°C may be 0.5 mm²/s or more, 0.8 mm²/s or more, or 1 mm²/s or more, and may be 10 mm²/s or less, 5 mm²/s or less, 3 mm²/s or less, 2 mm²/s or less, or 1.5 mm²/s or less.

A refractive index of the refrigerating machine oil at 20°C may be 1.445 or more, 1.450 or more, or 1.455 or more, and may be 1.480 or less, 1.470 or less, or 1.465 or less. When such a refrigerating machine oil is used, the coefficient of friction of the sliding portion tends to be lower than when using a mineral oil-based refrigerating machine oil that has a refractive index in this range but does not contain an alkylbenzene.

A refractive index (n20) of the refrigerating machine oil at 20°C and a kinematic viscosity (KV100) at 100°C preferably satisfy the following formula: $1.430 \leq n 20 - 0.002 \times KV 100 \leq 1.464 .$ Hereinafter, a value of "n20 - 0.002 × KV100" in the middle of the above formula is also referred to as an Nr value.

A lower limit of the Nr value in the above formula may be 1.430, 1.435, 1.440, or 1.445. An upper limit of the Nr value in the above formula may be 1.464, 1.462, 1.460, 1.459, or 1.458.

A pour point of the refrigerating machine oil may be 10°C or lower, 0°C or lower, -10°C or lower, -20°C or lower, -30°C or lower, or -40°C or lower. The pour point in the present specification means a pour point measured in conformity with JIS K2269:1987.

A density of the refrigerating machine oil may be, for example, 0.790 g/cm³ or more, 0.800 g/cm³ or more, or 0.810 g/cm³ or more, and may be 0.850 g/cm³ or less, 0.840 g/cm³ or less, or 0.835 g/cm³ or less. The density in the present specification means a density at 15°C measured in conformity with the "vibrating method" described in JIS K2249-1:2011.

The refrigerating machine oil can be present in the form of a working fluid composition in which the refrigerating machine oil is mixed with a refrigerant in a refrigeration machine having a refrigerant circulation system including a compressor, a condenser, an expansion mechanism, and an evaporator. That is, another embodiment of the present invention is a working fluid composition comprising the refrigerating machine oil described above and a refrigerant. A content of the refrigerating machine oil in the working fluid composition may be 1 part by mass or more or 2 parts by mass or more, and may be 500 parts by mass or less or 400 parts by mass or less, relative to 100 parts by mass of the refrigerant.

Examples of the refrigerant include hydrocarbons, saturated fluorocarbons, unsaturated fluorocarbons, fluorine-containing ethers such as perfluoropolyether, bis(trifluoromethyl) sulfide, trifluoroiodomethane, ammonia, and carbon dioxide.

The refrigerant preferably contains hydrocarbons. A content of the hydrocarbons may be 50% by mass or more, 60% by mass or more, 70% by mass or more, 80% by mass or more, 90% by mass or more, or 95% by mass or more, based on the total amount of the refrigerant. The refrigerant may consist only of hydrocarbons.

The hydrocarbons are preferably hydrocarbons having 1 to 5 carbon atoms, and more preferably hydrocarbons having 2 to 4 carbon atoms. Examples of the hydrocarbons include methane, ethylene, ethane, propylene, propane (R290), cyclopropane, normal butane, isobutane (R600a), cyclobutane, methylcyclopropane, 2-methylbutane, normal pentane, and mixtures of two or more of these. The hydrocarbons are preferably hydrocarbons that are gaseous at 25°C and 1 atm, and more preferably propane, normal butane, isobutane, 2-methylbutane, or mixtures thereof.

### Examples

Hereinafter, the present invention will be described more specifically based on Examples, but the present invention is not limited to the Examples.

In Examples and Comparative Examples, an alkylbenzene (a mixture of linear alkylbenzenes in which m and n in formula (1) are each independently integers of 1 to 6 and satisfy m + n = 9 to 12, average molecular weight: 242, kinematic viscosity at 40°C: 4.24 mm²/s, kinematic viscosity at 100°C: 1.42 mm²/s, refractive index: 1.483, N value: 1.480) and the following hydrocarbon oils 1 to 5 were used, and as one example, they were prepared so that kinematic viscosities at 40°C and 100°C became about 3 mm²/s and about 1.2 mm²/s, respectively.

### (Hydrocarbon oils)

Hydrocarbon oil 1: a mineral oil hydrocarbon oil obtained by fractionating, after hydrotreating, a hydrocracked light oil of a raw material containing a vacuum distillation residue oil (refractive index (20°C): 1.451, kinematic viscosity at 40°C: 2.39 mm²/s, kinematic viscosity at 100°C: 1.02 mm²/s, N value: 1.449, average molecular weight: 201, %C_{P}: 57.9, %C_{N}: 42.1, %C_{A}: 0, R_{N}: 1.06, R_{A}: 0.00, R_{T}: 1.06)

Hydrocarbon oil 2: a mineral oil hydrocarbon oil obtained by fractionating, after hydrotreating, a hydrocracked light oil of a raw material containing a vacuum distillation residue oil (refractive index (20°C): 1.443, kinematic viscosity at 40°C: 2.39 mm²/s, kinematic viscosity at 100°C: 1.04 mm²/s, N value: 1.441, average molecular weight: 204, %C_{P}: 75.8, %C_{N}: 23.7, %C_{A}: 0.5, R_{N}: 0.61, R_{A}: 0.02, R_{T}: 0.63)

Hydrocarbon oil 3: a normal paraffinic hydrocarbon oil obtained by adsorption separation with a molecular sieve and fractionation from a kerosene fraction obtained by hydrodesulfurizing a straight-run distillate oil of crude oil (refractive index (20°C): 1.429, kinematic viscosity at 40°C: 2.09 mm²/s, kinematic viscosity at 100°C: 0.97 mm²/s, N value: 1.427, average molecular weight: 201, %C_{P}: 99.7, %C_{N}: 0, %C_{A}: 0.3, R_{N}: 0.00, R_{A}: 0.01, R_{T}: 0.01)

Hydrocarbon oil 4: a mixture (mass ratio 50:50) of 1-tetradecene (reagent) and 1-hexadecene (reagent) (refractive index (20°C): 1.439, kinematic viscosity at 40°C: 2.21 mm²/s, kinematic viscosity at 100°C: 1.01 mm²/s, N value: 1.437, average molecular weight: 210, %C_{P}, %C_{N}, %C_{A}, R_{A}, and R_{N}: not applicable)

Hydrocarbon oil 5: an isoparaffin obtained by fractionating a paraffin component synthesized by a Fischer-Tropsch reaction from carbon monoxide and hydrogen after hydrogenolysis/isomerization/purification (refractive index (20°C): 1.432, kinematic viscosity at 40°C: 2.16 mm²/s, kinematic viscosity at 100°C: 0.96 mm²/s, N value: 1.430, average molecular weight: 204, %C_{P}: 97.2, %C_{N}: 2.6, %C_{A}: 0.2, R_{N}: 0.07, R_{A}: 0.01, R_{T}: 0.08).

After 1.5% by mass of tricresyl phosphate was blended into each of the alkylbenzene and the hydrocarbon oils 1 to 5 described above, a coefficient of friction was measured by the following procedure. The results are shown in Table 1.

### (Measurement of coefficient of friction)

Using an MTM (Mini Traction Machine) tester (manufactured by PCS Instruments), a coefficient of friction (µ) was measured under the following conditions. The results are shown in Table 1 and Table 2. A smaller coefficient of friction means that friction properties are superior.
Balls and disks: standard test pieces (AISI 52100 standard)
Test temperature: 40°C
Sliding speed: 0.3 to 0.9 m/s (partially extracted)
Load: 10 N
Slide-to-roll ratio: 30%
A value of |U_{D} - U_{B}| (m/s) was used as the sliding speed. Here, U_{D} is a speed (m/s) of a disk at the sliding portion, and U_{B} is a speed (m/s) of a ball at the sliding portion.

**[Table 1]**

| | | Alkylbenzene | Hydrocarbon oil 1 | Hydrocarbon oil 2 | Hydrocarbon oil 3 | Hydrocarbon oil 4 | Hydrocarbon oil 5 |
|---|---|---|---|---|---|---|---|
| | Sliding speed (m/s) | | | | | | |
| Coefficient of friction | 0.9 | 0.0169 | 0.0164 | 0.0102 | 0.0313 | 0.0089 | 0.0078 |
| | 0.75 | 0.0158 | 0.0156 | 0.0092 | 0.0317 | 0.0090 | 0.0076 |
| | 0.6 | 0.0157 | 0.0156 | 0.0091 | 0.0325 | 0.0098 | 0.0076 |
| | 0.45 | 0.0157 | 0.0158 | 0.0095 | 0.0337 | 0.0109 | 0.0084 |
| | 0.3 | 0.0164 | 0.0168 | 0.0104 | 0.0366 | 0.0137 | 0.0104 |

Subsequently, using the alkylbenzene and the hydrocarbon oils 1 to 5 described above, base oils having compositions (mass %) shown in Table 2 (based on the total amount of the base oils) were prepared. Each of the obtained base oils was blended with 1.5% by mass of tricresyl phosphate to obtain refrigerating machine oils of Examples and Comparative Examples. For each of the obtained refrigerating machine oils, a coefficient of friction was measured by the procedure described above. A value (µ - µ0) was obtained by subtracting the coefficient of friction (µ0) for the alkylbenzene shown in Table 1 from the coefficient of friction (µ) for each of the measured refrigerating machine oils, and a coefficient of friction reduction effect was evaluated on the basis of the value. Specifically, a negative value for (µ - µ₀) means that the coefficient of friction of the refrigerating machine oil containing the alkylbenzene and the hydrocarbon oil is reduced compared to that of the alkylbenzene alone, and a larger absolute value of this negative value means that the coefficient of friction reduction effect is large. The results are shown in Table 2.

**[Table 2]**

| | | | Comparative Example 1 | Example 1 | Example 2 | Example 3 | Example 4 |
|---|---|---|---|---|---|---|---|
| Composition of base oil (mass %) | Alkylbenzene | | 50 | 50 | 50 | 50 | 50 |
| | Hydrocarbon oil | 1 | 50 | - | - | - | - |
| | | 2 | - | 50 | - | - | - |
| | | 3 | - | - | 50 | - | - |
| | | 4 | - | - | - | 50 | - |
| | | 5 | - | - | - | - | 50 |
| Physical properties of refrigerating machine oil | Kinematic viscosity at 40°C (mm²/s) | | 3.1 | 3.1 | 2.9 | 3.0 | 3.0 |
| | Kinematic viscosity at 100°C (mm²/s) | | 1.2 | 1.2 | 1.2 | 1.2 | 1.2 |
| | Refractive index @20°C | | 1.468 | 1.462 | 1.455 | 1.460 | 1.458 |
| | Pour point (°C) | | <-45 | -32.5 | -2.5 | -17.5 | <-45 |
| | Density @15°C (g/cm³) | | 0.844 | 0.834 | 0.817 | 0.8239 | 0.820 |
| Coefficient of friction reduction effect µ - µ₀ | Sliding speed (m/s) | | | | | | |
| | 0.9 | | -0.0008 | -0.0039 | -0.0097 | -0.0102 | -0.0052 |
| | 0.75 | | -0.0001 | -0.0037 | -0.0095 | -0.0092 | -0.0041 |
| | 0.6 | | +0.0004 | -0.0018 | -0.0091 | -0.0094 | -0.0045 |
| | 0.45 | | +0.0012 | -0.0014 | -0.0093 | -0.0095 | -0.0040 |
| | 0.3 | | +0.0021 | -0.0022 | -0.0073 | -0.0078 | -0.0020 |

The Nr values of the refrigerating machine oils of Comparative Example 1 and Examples 1 to 4 are as follows.
Comparative Example 1: 1.4656
Example 1: 1.4596
Example 2: 1.4526
Example 3: 1.4576
Example 4: 1.4556

As can be seen from Table 2, in the case where the hydrocarbon oil 1 having a refractive index at 20°C exceeding 1.445 is mixed with the alkylbenzene (Comparative Example 1), almost no coefficient of friction reduction effect was obtained, whereas in the case where the hydrocarbon oils 2 to 5 having a refractive index at 20°C of 1.445 or less are mixed (Examples 1 to 4), a significant coefficient of friction reduction effect was obtained. In particular, in Examples 2 and 3, a remarkable coefficient of friction reduction effect (synergistic effect) was observed as compared with the alkylbenzene alone, the hydrocarbon oil 2 alone, or the hydrocarbon oil 3 alone.

Further, when the mass ratio of the above alkylbenzene (linear alkylbenzene) to each of the above hydrocarbon oils 2 to 5 is changed to 15/85, 30/70, 70/30, and 85/15, an additive or synergistic friction reduction effect is observed as compared with the alkylbenzene alone or each of the hydrocarbon oils 2 to 5 alone.

Further, when a branched alkylbenzene (having branched alkyl groups of carbon numbers 9, 12, and 15 derived from propylene oligomer) is used instead of the above linear alkylbenzene, although the coefficient of friction of the sliding portion tends to be higher than in the case of using the linear alkylbenzene, the coefficient of friction of the sliding portion can be reduced by mixing the hydrocarbon oils 2 to 5.

## Claims

1. A refrigerating machine oil comprising an alkylbenzene and a hydrocarbon oil other than the alkylbenzene, the hydrocarbon oil having a refractive index at 20°C of 1.445 or less.

2. The refrigerating machine oil according to claim 1, wherein a refractive index (n20) of the hydrocarbon oil at 20°C and a kinematic viscosity (KV100) at 100°C satisfy the following formula: $1.420 \leq n 20 - 0.002 \times KV 100 \leq 1.445 .$

3. The refrigerating machine oil according to claim 1, wherein a kinematic viscosity of the refrigerating machine oil at 40°C is 5 mm²/s or less.

4. A working fluid composition comprising the refrigerating machine oil according to any one of claims 1 to 3, and a refrigerant.

5. A method for reducing a coefficient of friction of a sliding portion by using a refrigerating machine oil containing an alkylbenzene, the method comprising mixing, with the alkylbenzene, a hydrocarbon oil other than the alkylbenzene, the hydrocarbon oil having a refractive index at 20°C of 1.445 or less, thereby reducing the coefficient of friction of the sliding portion.
